

Dec. 28, 1937.

R. E. FRICKEY

2,103,716

RAIL TREATMENT METHOD

Filed July 27, 1936

FIG. 1.



FIG. 4.



FIG. 5.



FIG. 6.



FIG. 2.



FIG. 3.



FIG. 7.



FIG. 8.



FIG. 9.

INVENTOR.  
Royal E. Frickey  
Paul D. Flehr  
ATTORNEY.

## UNITED STATES PATENT OFFICE

2,103,716

## RAIL TREATMENT METHOD

Royal E. Frickey, San Francisco, Calif., assignor  
to Welding Service, Inc., San Francisco, Calif.,  
a corporation of California

Application July 27, 1936, Serial No. 92,715

4 Claims. (Cl. 148—10)

This invention relates generally to methods and apparatus for hardening the ends of steel rails. More particularly it relates to heating operations to prepare rail ends for a hardening operation by 5 chilling.

It has previously been proposed to harden railroad rails, by heating the ends of the rails, followed by a chilling operation. The rail ends so treated, provided a proper degree and pattern of 10 hardness is secured, are better able to withstand the battering action of rolling stock, which in untreated rail sections invariably causes rapid deterioration of rail joints. In carrying out such processes, one problem involved is that of securing 15 rapid heating of a localized layer of the rail ball. In applying such operations at rolling mills, it is evident that time is an important factor, not only with respect to the cost of such operation, but also to maintain a production rate commensurate with 20 the capacity of the mill. Likewise, it has been found that unless the heating is carried out in such a manner as to produce uniform results in successive operations, it is difficult, if not impossible, to secure a uniform degree of hardness.

25 The present process and apparatus makes it possible to heat a localized layer of metal at the end of the rail section in a minimum period of time, and with such uniformity that subsequent controlled chilling operations will produce a relatively uniform degree of hardness.

Another object of the invention is to provide a rail heating method and apparatus which is relatively simple and convenient to apply, and which is well adapted for use by rolling mills.

35 Further objects of the invention will appear from the following description in which the preferred embodiment of the invention has been set forth in detail in conjunction with the accompanying drawing.

40 Referring to the drawing:

Fig. 1 is an end view showing apparatus incorporating the present invention, applied to a rail for heating the same, and also diagrammatically showing circuit connections.

45 Fig. 2 is a perspective detail diagrammatically illustrating the manner in which the magnetic flux is applied to the end of the rail.

Fig. 3 illustrates a temperature-time curve, for the type of heating which we employ.

50 Figs. 4 to 9 inclusive are cross-sectional views taken through a heated rail end, and showing the demarcation between metal heated to or above the critical temperature, and the remainder of the rail metal.

55 The present invention makes use of means for

producing an alternating magnetic flux, by use of an alternating current of more than standard frequency, as for example a frequency of about 500 cycles. This flux is applied to the ball of a rail, at one end of a rail section, and in such a 5 manner that the major part of the flux is concentrated in an upper layer of the ball. The rail ball is heated by eddy currents and hysteresis, with the major part of the heat being initially generated in the upper layer of the ball, until this 10 layer attains the critical temperature at which it is no longer magnetic. Thereafter application of the flux is continued, and for reasons to be presently explained, the upper layer of metal is heated to a temperature level substantially above the 15 critical temperature, as for example a temperature of about 1550° F., where the rail metal has a critical temperature of about 1350° F. The attainment of such a temperature level makes possible a convenient time lapse between termination 20 of the heating operation and the beginning of the chilling and quenching operation, and it also makes the entire process less critical, and thus facilitates the production of uniform results.

Referring now to the drawing, I have shown 25 what can be termed a transformer 10, and which consists of an inverted U-shaped magnetic core 11, the side legs of which are provided with windings 12. It is desirable to form the windings of metal tubing 13, which can be embedded in a 30 suitable refractory cement. In operation, cooling water or other suitable cooling fluid, is circulated through the windings, in order to maintain the various parts of the transformer below such temperature values as might cause failure. The end 35 portions 14 of the core are shown provided with oppositely bevelled faces 16, adapted to engage the upper side edges of the rail ball 17.

The exciting circuit for the transformer 10 can include an alternating current generator 18, delivering alternating current at a frequency of say 500 cycles per second, and capable of supplying a relatively large amount of electrical power, as for example from 15 to 25 kilowatts. In order to assist an operator in checking operation of the 45 transformer, the circuit is also shown including a volt meter 19, a watt-hour meter 21, and an ammeter 22. Also a condenser 23 is shown shunted across the windings of the transformer 10, in order to bring the power factor as near as possible to 50 unity.

Use of the equipment described above, and the carrying out of the present invention, can be described as follows:—Assuming that the ends 55 of 131 pound rails are to be heated, the electrical

power input to the transformer 10 can be about 18 kilowatts. The ends of the transformer core are seated upon the rail ball, in the manner illustrated in Figs. 1 and 2. Thus the core is 5 contacted with the upper part of the rail ball along two spaced lines, whereby the major part of the flux enters and leaves the rail along narrow zones located in the regions where the upper surface 24 of the rail ball merges with the side 10 ball faces 26. The length of these zones will of course depend upon the dimensioning of the core ends 14, although with a 131 pound rail, a length extending about three inches from the end of the rail, will suffice. It will be evident that heat 15 insulating material can be interposed between the core and the rail, to minimize transfer of heat into the core.

Current from the generator 18 is now applied to the transformer windings, to cause alternating 20 magnetic flux to thread laterally across the rail ball. While the entire rail ball forms a magnetic path through which the alternating flux traverses, the flux density is by far greatest in the upper layer of the rail ball, since this upper layer forms 25 the shortest path between the pole ends 14. Because of this greater flux density, and also because of so-called skin effect, a greater amount of heat is developed in this upper zone of the ball, including heating by virtue of flow of eddy currents, 30 and heating by hysteresis loss. Thus the upper portion of the rail ball is rapidly heated to the so-called critical temperature, at which the steel of the rail no longer is magnetic.

The magnetic flux now becomes denser in the 35 lower portions of the rail ball, underlying the portions which have been heated to the critical temperature, and although the flux density in the upper layer of heated metal is greatly reduced, heat in this upper layer continues to be generated, by virtue of flow of eddy currents through 40 the same. Thus with apparatus capable of maintaining the total amount of magnetic flux substantially constant throughout a heating period, it is possible to carry the temperature of the upper 45 ball portion to a value considerably above the critical temperature, while the underlying portion of the ball remains magnetic.

After a given period of time, such a period of 50 about 80 seconds for the representative example cited above, the upper layer of metal will have attained a temperature in the neighborhood of 1550° F. The transformer is then removed, and the upper surface of the rail end is chilled in a manner calculated to produce a predetermined 55 degree of hardness. For example the upper surface of the rail end can be contacted with a chilling liquid like water, applied at the end of a predetermined interval following discontinuance of heating, and with other factors controlled in 60 such a manner as to produce absorption of a predetermined amount of heat.

The curves of Fig. 3 serve to illustrate how my 65 method differs from other induction heating methods employing a circuit of magnetic material. Curve *a* represents a typical induction heating of a mass of steel in a circuit of magnetic material, where a magnetic flux is threaded relatively uniformly throughout the body. It 70 will be noted that the temperature rapidly rises to the critical value at about 1350° F., and thereafter the temperature-time curve flattens out, showing that there is no further increase in temperature. While it is possible to harden steel heated to a temperature of 1350° F., any such 75 process will be highly critical, due to the fact that

a slight lowering of the temperature below such value before the chilling operation, will cause a wide variation in the degree of hardness produced. The type of heating which I utilize is 5 illustrated by curve *b*, which changes its slope at the critical temperature, but which shows a continued rise in temperature as the heating operation is continued. This curve *b* was plotted with an electrical input of about 18 kilowatts, and with a temperature being measured at a 10 point about  $\frac{1}{4}$  inch below the upper surface of the rail ball, near the end of the rail being heated. It will be noted in connection with this curve that the critical temperature was reached in about 35 seconds following commencement of the heating 15 operation, and that in about 100 seconds the curve reached an elevated temperature of about 1590° F., and commenced to flatten out, showing that a further extension of the heating period would not be productive of a materially higher 20 temperature. I am of the opinion that the successful features of my method can be attributed largely to the discovery of a proper procedure to carry the temperature of the upper surface of the rail beyond the critical value, as exemplified 25 by this curve *b*, and by the use of electrical induction employing a circuit of magnetic material.

Figures 4 to 9 inclusive illustrate the localized character of the heating, in a typical instance. In these figures the dotted lines 1 to 6 inclusive 30 represent the line of demarcation between the upper layer of metal heated above the critical temperature, and the underlying layer of metal which is below the critical temperature. Fig. 4 represents the end face of the rail, while the sub- 35 sequent figures represent transverse sections taken at consecutive positions extending back from the end of the rail, and spaced one-half inch apart. Note that for a substantial distance back from the end of the rail, an upper layer of 40 metal is provided which is heated to or above the critical temperature. It will also be evident from these figures that chilling can be carried out to harden the side faces of the ball as well as the upper surface, or to harden only a limited zone 45 in the upper surface of the ball.

Previous mention has been made of the desirability of controlling both the heating and chilling operations, to produce uniformity in successive hardening operations. With the type of 50 heating described, it has been found possible to successively heat rail ends within remarkable close limits, as for example the limits of plus and minus 10° F. In practice, the generator 18 is constructed and operated to produce a fairly 55 constant output. From the time current is applied to the transformer 10, the operator determines the end of the heating period by observing the watt-hour meter 21, or this watt-hour meter can be provided with an automatic means, 60 whereby after a predetermined amount of energy has been supplied, the current is automatically interrupted. Uniformity of the quenching operation can be secured by maintaining certain factors constant. For example the chilling liquid is applied to the heated portion of the rail at the end of a predetermined time interval, following the heating operation. Likewise the chilling liquid is maintained at a constant temperature for successive operations, and is applied for a determined 65 time interval. It should also be applied in such a manner as to be conducive to uniform absorption of heat, as for example by causing a stream of the chilling liquid to flow over the heated surface of the rail at a predetermined velocity. 70 75 76

I claim:

1. In a method of heating steel rail ends preparatory to hardening the same by chilling, placing an upper layer of the rail ball, at one end of the rail, in a magnetic flux path, causing an alternating magnetic flux to thread said path to heat said layer to a temperature corresponding to the critical temperature of the rail metal, and thereafter continuing to heat said layer to a temperature materially above said critical temperature value by causing the major portion of said flux to pass through lower magnetic strata of the rail ball.
2. In a method of heating steel rail ends preparatory to hardening the same by chilling, placing an upper layer of the rail ball at one end of the rail in a magnetic flux path, causing an alternating magnetic flux to thread said path to inductively heat said layer to a temperature corresponding to the critical temperature of the rail metal, said magnetic flux entering and leaving the rail ball at spaced zones located at the upper side edges of the rail ball, and thereafter continuing application of said alternating magnetic flux to thereby continually heat said layer to a temperature materially above said critical temperature value, with passage of a major part of the magnetic flux through progressively lower magnetic strata of the rail ball.
3. In a method of heating steel rail ends pre-

paratory to hardening the same by chilling, placing an upper layer of the rail ball, at one end of the rail, in a magnetic flux path, causing an alternating magnetic flux to thread said path to heat said layer to a temperature corresponding to the critical temperature of the rail metal, thereafter continuing to heat said layer to a temperature materially above said critical temperature value by causing the major portion of said flux to pass through progressively lower strata of the rail ball, 10 and discontinuing the passage of magnetic flux after a predetermined amount of electrical energy has been consumed.

4. In a method of heating steel rail ends preparatory to hardening the same by chilling, placing an upper layer of the rail ball, at one end of the rail, in a magnetic flux path, the path extending laterally across the rail between the upper parallel side edges of the rail ball, causing an alternating magnetic flux to thread said path 20 to heat said layer to a temperature corresponding to the critical temperature of the rail metal, the major part of the flux entering and leaving said rail along narrow zones substantially coincident with said side edges, and thereafter continuing to 25 subject the rail ball to said magnetic flux without a material shift in said zones, to heat the upper layer to a temperature materially substantially above said critical temperature.

ROYAL E. FRICKEY.